

April 30, 1940.

N. OBENSHAIN ET AL

2,199,228

METHOD OF AND APPARATUS FOR COATING PAPER

Filed July 16, 1936



INVENTORS  
NOEL OBENSHAIN  
WRIGHT M. WELTON  
BY *S. E. Berry*  
ATTORNEY

## UNITED STATES PATENT OFFICE

2,199,228

METHOD OF AND APPARATUS FOR  
COATING PAPER

Noel Obenshain and Wright M. Welton, Piedmont, W. Va., assignors to West Virginia Pulp and Paper Company, New York, N. Y., a corporation of Delaware

Application July 16, 1936, Serial No. 90,832

6 Claims. (Cl. 91—50)

Our present invention relates to methods of and apparatus for coating paper.

The coating of paper with suspensions of mineral pigments, to which this application particularly applies, has presented serious problems for the reason that such suspensions commonly used in the paper art do not of themselves smooth out when applied with even slight irregularities. When the paper is coated by a direct application of the coating liquid there are formed, unless special precautions are taken, ripples or irregularities of the coating material on the paper which, when dried, produce streaks. Therefore, in much of the prior art practice, provision is made for smoothing out the ripples or other irregularities formed upon application, either by the use of reciprocating brushes or of smoothing or trowelling rolls. Such aids, however, have the drawbacks that they are cumbersome and are responsible for a comparatively low rate of output.

In view of these difficulties, proposals have been made to apply a measured amount of coating material upon the travelling sheet of paper to be coated, in such manner as to produce an even coating in the first instance and thus obviate the use of subsequent smoothing devices. It is to this latter class of coating methods and apparatus that our present invention is directed, and it is a principal object thereof to devise a new method and apparatus which will produce a coating of the usual mineral or other pigments having in a high degree the qualities of smoothness and uniformity, and in addition having the advantages of high output and reliability of operation.

In carrying out our invention we make use of coating rolls having cut or formed therein a multitude of liquid receiving indentations or grooves, such rolls being preferably of metal and having the surface thereof formed either by mechanical cutting or by photo engraving or other processes known to that art.

Our invention will be best understood by reference to the following detailed description taken with the annexed drawing in which:

Fig. 1 shows diagrammatically an arrangement of coating rolls constituting a preferred embodiment of our invention.

Fig. 2 is a side view of same.

Fig. 3 is a view of a roll in which the grooves are of the screen type.

Fig. 4 is a view of a roll in which the grooves 55 are of the inclined parallel type.

Fig. 5 shows an arrangement for coating both sides of the paper in one operation; and

Fig. 6 is a side view of same.

In Fig. 1 the coating material is sprayed through pipe 9 upon the coating roll 12 of the type shown in Figs. 3 or 4 to be more fully described hereinafter. The excess coating is caught in pan 10 and is pumped therefrom back to the spray pipe 6 by means not shown. Roll 12 is driven from a source not shown and has in contact therewith an offset or applicator roll 14 which may be driven simply by contact with roll 12 or preferably is positively driven by means of gears 13 and 13a shown in Fig. 2 which operate to drive said rolls at the same surface speed. The coating material fills to excess the multitude of pockets or grooves in the surface of the roll 12 and a portion of the liquid so picked up is transferred to the offset roll 14, which has a resilient surface as of rubber, the excess coating being squeezed out by the contact or nip between rolls 12 and 14, so that roll 14 acquires a uniform amount of coating for each contact with the roll 12 without the use of a doctor roll or blade. The so-coated surface of the roll 14 then is brought in contact with the paper web 16 which passes over the roll 14 and is held in proper juxtaposition with respect to roll 14 by means of the guide rolls 17, 18 and 19. As revealed by Fig. 1, the transfer or offset roll 14 moves in a direction 10 reverse to the travel of the web 16.

Various factors govern the uniformity of coating imparted to the web 16. One of these is the amount of slip between the web and the offset roll 14. For convenience this slip may be reckoned as the algebraic difference between the speeds of the web and the roll 14 divided by the speed of the paper and multiplied by 100 to give a percentage ratio, a direction of rotation of the roll reverse to the web being considered negative. Thus far we have found that satisfactory results are had when the percent slip for the arrangement of Fig. 1 is between 200 and 450. These conditions, for example, will be fulfilled when the paper has a speed of 500 feet per minute and the roll a speed in reverse of the paper of 600 feet per minute, thereby giving a percent slip of 220. Another factor is the nature and frequency of the markings on the roll 12. Good results have been obtained when a screen marking has been used of a frequency of 25 to 150 lines per inch, such a roll being shown in Fig. 3. The use of the parallel line marked roll of the type shown in Fig. 4 has given results as good as, if not better than, those obtained with the 55

screen marking. In the roll of Fig. 4 the grooves 25 have a pitch of approximately 30 degrees to the axis of the cylinder. The number of lines per inch may vary from 25 to 150 more or less 5 with a groove to wall thickness ratio of from 3 to 1 to 4 to 1; it being understood that the above figures are given by way of example without limiting the invention to any exact size or arrangement of markings. The indented rolls may 10 desirably be made of copper or other non-corrod- ing metal, and if desired may be chromium plated. Non-metallic indented rolls might also be em- ployed. Such rolls in general may be made in a manner similar to the manufacture of the in- 15 taglio cut rolls used in rotogravure printing. The amount of coating applied may be best regulated either by varying the consistency of the coating or by choosing rolls of varying depth of cut or by varying both these factors.

20 Thus far when using the usual mineral pig- ments or fillers we have obtained superior results by driving the offset roll in a direction reverse to the travel of the paper, in comparison with those obtained by driving the offset roll in the same di- 25 rection as the paper. However, in some instances satisfactory results may be had when driving the offset roll in the same direction with the paper, especially when using coating compositions hav- 30 ing greater coating or spreading power than those commonly used for coating paper. When the offset roll is rotated in the same direction as the paper, considerable slippage should be had, as, for example, in the neighborhood of +60 per cent., the positive slip indicating that the paper moves 35 faster than the surface speed of the applicator roll.

When it is desired to coat both sides of the sheet in the same operation, an arrangement of parts may be employed as illustrated in Figs. 5 and 6.

40 After being coated the paper is then passed through a drying chamber, as is common in the art.

In lieu of spraying the coating upon the in- 45 dented roll, as by the spray pipe 9, the composition may be fed to the pan 10 and the latter raised so as partially to immerse the roll 12.

The improved method and apparatus described 50 in the foregoing is adapted to be used with a variety of paper coating compositions. Typical compositions containing in suspension the usual mineral fillers or pigments are as follows:

(1) Chalk----- 100 parts  
Casein----- 15 to 18 parts  
55 Water added to give----- 35% solids

The mixture is then ground through a 3 roll ink grinder, diluted to 25% solids and re-ground.

(2) Clay----- 500 parts  
60 Satin white----- 850  
Chalk----- 150  
Casein----- 215  
Water added to give----- 20% solids

65 and suitably ground. By varying the amount of solids in suspension and the depth of grooving on the indented rolls as aforesaid, coatings of the type of the above examples have been successfully applied ranging from .3 pound to 10 pounds per 70 ream per side.

This amount of coating seems not to vary ap- 75 preciably with the degree of wrap of the paper around the applicator roll. Furthermore, slight variations in the degree of slip have very little effect on the amount of composition applied. The

improved process has thus far enabled us to coat paper at a surface speed as low as 100 to as high as 500 feet per minute.

Our improved method and apparatus may be used to coat paper previously formed and dried, 5 or it may be used to coat the paper while the latter is in the paper making machine and before the web has been fully dried.

In the claims, by "paper" is meant to include cardboard or pasteboard or other paper products 10 which it may be desired to coat.

Various changes from the detailed description and specific data above given will occur to those skilled in the art, without, however, departing from the spirit of the invention or the scope of 15 the appended claims.

We claim:

1. The method of coating a web of paper or the like, which comprises applying a coating composition comprising mineral pigments to a cylind- 20 rical surface having a multitude of liquid receiv- ing indentations serving to hold a measured quantity of such composition, transferring a portion of said coating so applied to a second surface having resilient properties by maintaining said surfaces 25 in rolling contact whereby said resilient surface receives a uniform amount of coating composi- tion which is less than the amount initially pres- ent on said surface having indentations, then 30 contacting said resilient surface with a web of 30 paper or the like moving with respect to said resilient surface so as to occasion a substantial slip between said web and said contacting sur- face, while maintaining said web free to move slight amounts incident to variations in diameter 35 and position of said resilient cylindrical surface.

2. The method according to claim 1 in which said slip varies from 200% to 500%.

3. The method of coating a web of paper or the like, which comprises applying a coating com- 40 position comprising mineral pigments to a cylind- rical surface having a multitude of liquid receiv- ing indentations, transferring a portion of said coating so applied to a second surface having resilient properties by maintaining said surfaces 45 in rolling contact whereby said resilient surface receives a uniform amount of coating composi- tion which is less than the amount initially pres- ent on said surface having indentations, then 50 contacting said resilient surface with a web of 50 paper or the like moving in the reverse direction to said resilient surface, while maintaining said web free to move slight amounts incident to variations in diameter and position of said resil- 55 ient cylindrical surface.

4. In a device adapted for coating paper with a liquid suspension of finely divided mineral pig- ments or fillers, a roll comprising a cylindrical 60 surface having a multitude of liquid receiving in- dentations, means for supplying the coating com- position to said roll, a resilient transfer roll re- ceiving coating from said indented roll and ap- 65 plying same to a paper web, means for driving said transfer roll in reverse direction to the travel of said web, guide rolls for passing the paper over 70 said transfer roll, said guide rolls being disposed so as to permit the paper to maintain contact with the transfer roll regardless of minute variations in the position of said roll.

5. In a device adapted for coating paper with 70 a liquid suspension of finely divided mineral pig- ments or fillers, a roll comprising a cylindrical 75 surface of relatively hard material having liquid receiving indentations of a frequency from 25 to 150 per inch, means for supplying the coating 75

composition to said roll, a resilient transfer roll rotating in contact with said indented roll and receiving coating from said indented roll and applying said coating to a paper web, and means 5 for driving said transfer roll in reverse direction to the travel of said web.

6. In a device adapted for coating paper with a liquid suspension of finely divided mineral pigments or fillers, a roll comprising a cylindrical 10 surface having a multitude of liquid receiving indentations, means for supplying the coating composition to said roll, a resilient transfer roll

receiving coating from said indented roll and applying same to a paper web, means for driving said transfer roll in reverse direction to the travel of said web, and means for driving said indented roll and said transfer roll at substantially the 5 same surface speed, guide rolls for passing the paper over said transfer roll, said guide rolls being disposed so as to permit the paper to maintain contact with the transfer roll regardless of minute variations in the position of said roll. 10

NOEL OBENSHAIN.

WRIGHT M. WELTON.